

[54] ELECTRIC INCANDESCENT LAMPS

[76] Inventors: John Michael Rees; George Eric Coxon; Robert Bernard Johnston, all of Thorn House, Upper St. Martin's Ln., London WC2H 9ED, England

[22] Filed: May 29, 1973

[21] Appl. No.: 364,917

## Related U.S. Application Data

[63] Continuation-in-part of Ser. No. 317,813, Dec. 22, 1972, abandoned.

[52] U.S. Cl. .... 313/222, 316/20

[51] Int. Cl. .... H01k 1/50, H01k 3/00

[58] Field of Search.... 313/222; 316/20

## [56] References Cited

## UNITED STATES PATENTS

3,712,701 1/1973 Johnson et al. .... 313/222

3,738,729 6/1973 Coxon et al. .... 313/222

Primary Examiner—Herman Karl Saalbach

Assistant Examiner—Darwin R. Hostetter

Attorney, Agent, or Firm—Kemon, Palmer and Estabrook

## [57] ABSTRACT

A tungsten-halogen cycle electric incandescent lamp contains a solid aromatic halide in the fill which dissociates when the lamp is heated to provide halogen to support the regenerative cycle. The aromatic halide can be hexabromobenzene or hexachlorobenzene and the fill may also include a halophosphonitrile.

## 11 Claims, 3 Drawing Figures



PATENTED MAY 14 1974

3,811,063

FIG. 1.



FIG. 2.



FIG. 3.



## ELECTRIC INCANDESCENT LAMPS

This application is a continuation-in-part of our application Ser. No. 317,813 filed Dec. 22nd, 1972, now abandoned.

The present invention relates to tungsten-halogen electric incandescent lamps.

Such lamps have a tungsten filament enclosed within a light-transmitting envelope containing a fill of non-reactive gas, such as N<sub>2</sub>, Ar, Kr or Xe and a small quantity of halogen, for example iodine.

The simplified mechanism of the reactions occurring during operation of such a lamp is that tungsten escaping from the incandescent filament, which would normally diffuse to the bulb wall, reacts with the iodine to form tungsten iodide. When the tungsten iodide diffuses into the high temperature zone surrounding the filament it dissociates, liberating the tungsten and iodide. This regenerative cycle effectively prevents radial diffusion of tungsten, and the bulb wall remains clean throughout life. Consequently, bulb surface area is not important in a lamp where a regenerative cycle is operating and this allows very compact lamps with mechanically strong tubular fused silica envelopes to be used, so permitting filling to a pressure of several atmospheres, which gives improved filament life.

More recently, bromine has been used in place of iodine but while this eliminated the characteristic mauve tinge caused by the selective absorption of molecular iodine, it was found that precise control was required to avoid reaction between excess bromine and solid tungsten. It was shown that this reaction could be inhibited by introducing hydrogen, and HBr, CHBr<sub>3</sub>, CH<sub>2</sub>Br<sub>2</sub> and CH<sub>3</sub>Br were suggested as a suitable means of transporting hydrogen and bromine into a lamp, but this has the disadvantage that diffusion of hydrogen through fused silica may result in an excess of free bromine in a lamp during its life, which causes tungsten erosion and eventual failure. In consequence it is usual to employ iodine in long life lamps (above 1,000 hours) and bromine, admitted as a hydrogen-containing compound, in shorter life lamps.

The disadvantage of gaseous halogen dosing, and in particular the use of hydrogen-containing halides, was discussed in U.S. Pat. application Ser. No. 1404, now abandoned which proposed the use of halophosphonitriles as a halogen source.

It has now been found, according to the present invention, that solid aromatic organic halides represent a useful means of introducing halogen into a tungsten-halogen incandescent lamp. Suitable aromatic halides have a low vapour pressure and preferably introduced into the lamp envelope as a solution in a volatile non-polar solvent, such as petroleum-ether (especially 60°-80° C b pt), ether, and cyclic, aromatic or chlorinated hydrocarbons, e.g. benzene which is removed from the lamp by evacuation or by flushing with a dry non-reactive gas, (e.g. nitrogen).

Of particular interest for the purposes of this invention are hexahalogenated benzenes, and especially hexabromobenzene and hexachlorobenzene.

Dosing with hexachlorobenzene has been found to be particularly useful with short life film projection lamps having an operational filament temperature of more than 3,000° K and a life of up to 100 hr.

The advantages of the use of solid aromatic halides include accuracy and repeatability of dosing, relative

insensitivity to moisture and the reduction, and in some cases elimination, of hydrogen from the cycle.

Tungsten-halogen lamps in accordance with the invention will now be more fully described by way of example only with reference to the accompanying drawings, in which:

FIG. 1 shows a completed two-ended tungsten-halogen lamp; and

FIGS. 2 and 3 show a single-ended lamp and a U-shaped lamp, respectively, in the course of manufacture.

Referring to the accompanying drawings, like reference numerals indicate similar portions of the lamps.

In each of the lamps shown, there is a quartz envelope 1 surrounding a tungsten filament 2, with lead-in wires 4, which are press-sealed through the ends of the envelope 1, for supplying electrical current to the filament 2.

In the lamp shown in FIG. 1, the filament 2 is mounted on filament supports 3 within the envelope 1, and the ends of the lamp have contact members 5 connected to the lead-in wires 4. The envelope 1 contains nitrogen, carbon and a halogen the carbon and halogen having been formed by the thermal dissociation of a solid aromatic halide, e.g. a hexahalogenated benzene within the lamp envelope 1.

In the lamps shown in FIGS. 2 and 3 the filament 2 is connected to electrically conductive foils 6 press-sealed within the material of the lamp envelope 1, and the foils 6 are in turn connected to the lead-in wires 4. The envelopes 1 each have exhaust tubes 7 connected thereto, giving access to the interior of the envelope.

In FIG. 3, the lamp has within the envelope 1 filament supports 3 on which the filament 2 is mounted.

Examples of methods of making lamps according to the invention will now be described.

A typical example of the practice of this invention is the dosing with hexabromobenzene of a 12V 55W single end automobile lamp of the type shown in FIG. 2. The needle of a hypodermic syringe is inserted into the unsealed exhaust tube 7 of the lamp, and 0.025 cm<sup>3</sup> of a solution containing 0.05g of hexabromobenzene in 100 cm<sup>3</sup> of benzene is injected into the envelope 1. The solvent is removed by flushing with a stream of dry nitrogen (preferably containing less than 10 ppm of water vapour) passed through the exhaust tube 7, after which the envelope 1 is exhausted and gas-filled with a non-reactive gas such as N<sub>2</sub>, Ar, Kr or Xe in the usual manner, and the exhaust tube 7 is sealed off. On operation of the lamp, or otherwise raising it to a high temperature, the hexabromobenzene dissociates to yield bromine for supporting the regenerative cycle.

In a further example, a 12V, 100W single-ended projection lamp of the type shown in FIG. 2, having a nominal efficiency of 30 lm/W and a rated life of 25 hours, is produced using hexachlorobenzene as the dosing substance. The needle of a hypodermic syringe is inserted into the unsealed exhaust tube 7 of the lamp, and 0.05 cm<sup>3</sup> of a solution containing 0.04g of hexachlorobenzene in 100 cm<sup>3</sup> of toluene is injected into the envelope 1. The solvent is then removed by flushing with a stream of dry nitrogen with the bulb temperature raised to 100° C to speed up the extraction process. After this the envelope is exhausted and gasfilled with a non-reactive gasfilling in the usual manner.

A further advantage of aromatic halides is that they are compatible with halophosphonitriles (the use of

which is described in the above-mentioned patent application Ser. No. 1,404). A mixture of these can be added to a lamp either as separate solutions or as a mixture in a single solution. This enables the ratio of phosphorus to halogen to be regulated to suit the particular lamp, or a mixture of halogens to be added in accurately controlled proportions.

One example of this aspect of the invention is in the production of a 240V 1,000W photographic U-lamp type of the type shown in FIG. 3. Such a lamp can be made by dispensing 0.05 cm<sup>3</sup> of a solution containing 0.1g of bromophosphonitrile and 0.1g of hexabromobenzene in 100 cm<sup>3</sup> of benzene into the lamp by way of the exhaust tube 7. Again, the solvent is removed by flushing with a stream of dry nitrogen followed by exhaustion and gas-filling with a non-reactive gas.

We claim:

1. A tungsten-halogen cycle electric incandescent lamp comprising: a light-transmitting, high temperature-resisting envelope; a tungsten filament within said envelope; lead-in wires sealed through said envelope and connected to said filament; and a fill within said envelope capable of supporting a tungsten-halogen regenerative cycle in co-operation with said filament, said fill comprising a non-reactive gas, carbon, and a halogen, said carbon and halogen having been formed by dissociation of a solid aromatic halide within said envelope.

2. A lamp as claimed in claim 1 wherein said fill includes hydrogen formed by dissociation of said halides.

3. A tungsten-halogen cycle electric incandescent lamp comprising: a light-transmitting high temperature-resisting envelope; a tungsten filament within said envelope; lead-in wires sealed through said envelope and connected to said filament; and a fill within said envelope comprising a non-reactive gas and a solid aro-

matic halide.

4. A lamp as claimed in claim 1 wherein said carbon, and halogen have been formed by dissociation of a halogenated benzene.

5. A lamp as claimed in claim 4 wherein said halogenated benzene is a hexahalogenated benzene.

6. A lamp as claimed in claim 5 wherein said hexahalogenated benzene is hexabromobenzene.

7. A lamp as claimed in claim 5 wherein said hexahalogenated benzene is hexachlorobenzene.

8. A lamp as claimed in claim 1 wherein said fill includes a halogen, phosphorus and nitrogen formed by dissociation of a halophosphonitrile within said envelope.

9. A method of making a tungsten-halogen cycle electric incandescent lamp comprising the steps of:

providing a light-transmitting high-temperature resisting envelope having an aperture therein, a tungsten filament therewithin, and lead-in wires connected to said filament and sealed therethrough; introducing a normally solid aromatic halide into said envelope through said aperture; exhausting said envelope; gas-filling said envelope with a non-reactive gas; sealing said aperture; and raising said envelope to a high temperature sufficient to dissociate said aromatic halide.

10. A method as claimed in claim 9 wherein a solution of a solid aromatic halide in a volatile non-polar solvent is introduced into said envelope, said solvent being volatilised from said envelope before said gas-filling step.

11. A method as claimed in claim 9 wherein said solvent is selected from the group consisting of petroleum ether; cyclic hydrocarbons; aromatic hydrocarbons and chlorinated hydrocarbons.

\* \* \* \* \*

UNITED STATES PATENT OFFICE  
CERTIFICATE OF CORRECTION

Patent No. 3,811,063

Dated May 14, 1974

Inventor(s) John Michael Rees, George Eric Coxon, Robert  
Bernard Johnston

It is certified that error appears in the above-identified patent  
and that said Letters Patent are hereby corrected as shown below:

[30] Foreign Application Priority Data

June 12, 1972 Great Britain ..... 27408/72

Signed and sealed this 10th day of September 1974.

(SEAL)  
Attest:

McCOY M. GIBSON, JR.  
Attesting Officer

C. MARSHALL DANN  
Commissioner of Patents